

# UNITED STATES PATENT OFFICE.

ARTHUR D. LITTLE, OF PROVIDENCE, RHODE ISLAND, ASSIGNOR TO JOHN T. WHEELWRIGHT, OF BOSTON, MASSACHUSETTS.

## LINING FOR DIGESTERS.

SPECIFICATION forming part of Letters Patent No. 351,330, dated October 19, 1886.

Application filed June 7, 1886. Serial No. 204,371. (No specimens.)

*To all whom it may concern:*

Be it known that I, ARTHUR D. LITTLE, of Providence, Rhode Island, have invented a new and useful Improvement in Linings for 5 Digesters, of which the following is a specification.

My invention relates to wood-pulp digesters made of cast-iron, in which the so-called "acid" or "bisulphite" processes are employed, and 10 has still more especial reference to a lining for the same. These digesters are commonly lined with sheet-lead, first, to protect the iron of which the shell is made from the corrosive action of acids used or evolved in the manufacture 15 of wood pulp by the process named above, and, secondly, to prevent discoloration of the pulp by the salts of iron otherwise formed. In use the lead lining presents certain difficulties and objections which it is the 20 object of my invention to remove. Lead expands in heating more than iron, and on the cooling down of the digester the lead lining, when in the form of sheets, does not contract sufficiently to return to place, and after several 25 operations the lead, especially at its place of fixed connection with the digester side, is thinned out by these alternate expansions and partial contractions, and finally cracks and breaks, no longer insuring the contents from 30 direct contact with the walls of the digester. Owing to these peculiarities of the lead linings now in use, constant watchfulness and care are required, and the work of repair is both expensive and tedious. I have found by experiment 35 that an oxide of lead, as litharge, may be applied to the inner surface of the digester in the form of an enamel or glaze, which will retain all the advantages of the sheet-lead lining in preventing chemical action between 40 the iron walls or shell of the digester and its contents, while at the same time it does not possess the disadvantages of sheet-lead hereinabove enumerated. In carrying out my invention I employ borate of lead and litharge. 45 Various methods of applying the compound to the digester as a lining will doubtless suggest themselves to builders of digesters, according to circumstances. There are but two principal difficulties to be overcome. First,

the liability of the compound to form bubbles, 50 and, second, the great heat to which the workmen are exposed.

My process has been as follows: The litharge and borate of lead are carefully ground and mixed together in the proportions of about 55 ten pounds of the former to one of the latter. The mixed powder is then melted in a pot so constructed that the gas from the fire cannot come in contact with the contents of the pot on account of its reducing action. The powder itself is such a poor conductor of heat that I have found it necessary to bring all parts of the melting-pot to a red heat and to stir the mixture constantly. After the mixture is thoroughly melted the pot is removed from the 65 furnace and allowed to stand until the mixture, constantly stirred meanwhile, is free from bubbles, when it is slowly poured into a heavy mold, the bottom of which has the shape of the digester-section that is to be coated. Both 70 the melting and the cooling should be done as quickly as possible to prevent the reduction to lead.

To separate from the mixture any reduced lead formed in the melting, the pot, near its 75 bottom, is provided with a ledge, which keeps back the heavy reduced lead when the melted mixture is poured out into the mold. After the cake which forms in the mold is removed therefrom it is clamped within an iron band, 80 and thus clamped is provided with long handles by which it may be manipulated, as presently set forth, without exposing the workmen to an unbearable degree of heat. In the meantime the section of the digester which is to be lined 85 is mounted upon slowly-revolving rollers and heated to a red heat by jets of gas mixed with air to burn with a blue flame, the number and size of the jets depending upon the weight of the casting. The cake is now introduced 90 axially through the section to be lined and pressed down by the handles, the workmen standing on either side. This continues until the slowly-revolving casting has melted off from the cake and received a uniform coating 95 or lining. Such portions of the edges of the casting as are not affected by the process thus far described are coated by a lump of the

mixed material of any shape that will allow it to be held in tongs or any suitable instrument.

In practice the end sections of the digester 5 may be lined with sheet-lead.

It is obvious that by observing proper proportions other oxides of lead may be substituted for the litharge, since they necessarily reduce to litharge in following the process.

10 The same is true of carbonate of lead and nitrate of lead.

In practical use the lining of the digester thus formed works in the same manner as an ordinary lead lining—that is, after a few boilings there is formed upon either lining a sur- 15

face coating of sulphate of lead, which, while it is harmless to act upon the wood treated in the digester, protects the glaze of my lining just as it protects the sheet-lead of the ordinary lining.

20

I claim—

A cast-iron digester the inner surface of which is coated with a glaze consisting of oxide of lead and borate of lead, substantially as described.

ARTHUR D. LITTLE.

Witnesses:

W. W. SWAN,  
WM. S. ROGERS.